

## UNITED STATES PATENT OFFICE.

CARL BACHE-WIIG, OF PORTLAND, MAINE; BERTHA M. BACHE-WIIG EXECUTRIX OF  
SAID CARL BACHE-WIIG, DECEASED.

## METHOD OF PREPARING PULP.

No Drawing. Application filed April 27, 1918, Serial No. 231,204. Renewed December 22, 1919. Serial No. 346,769.

*To all whom it may concern:*

Be it known that I, CARL BACHE-WIIG, a citizen of the United States, a resident of Portland, in the county of Cumberland and 5 State of Maine, have invented an Improvement in Methods of Preparing Pulp, of which the following is a specification.

This invention has for its object the production of pulp by a novel method, from 10 straw, corn-stalks, wood, baggasse and similar cellulosic substances, wherein the ligneous matter is retained for the most part in order that its weight may be added to the mass; and also the pulp can be bleached so 15 that it may be used for a fine grade of paper as well as for news print and other lower grades. Certain features of this invention are disclosed in my Patent No. 1,327,221, issued January 6, 1920.

20 My novel method involves two treatments which are preferably carried on successively.

By my first treatment the cellulosic material composing the pulp is softened, that is to say, its ligneous matter is softened but 25 not destroyed and its fibers are swollen and caused to separate.

In carrying out the first treatment I may proceed as follows:—the material or substance employed, in small pieces, or cut into 30 suitable short lengths, is placed in a tank or digester, which may be open or closed, and a softening agent, a solution of sodium chloride. (NaCl) is added, as for instance, I may add water containing from one half 35 of one to three percent of sodium chloride; and then heat the mass to a temperature of from 70° C. to 110° C. for from 12 to 72 hours, the temperature and time being more or less variable depending on the materials 40 used and the strength thereof, yet it will be understood that ordinarily the higher the temperature the shorter the time required, and vice versa. During this first treatment the ligneous matter and fiber, are acted 45 upon and gently softened but not destroyed.

The ligneous matter may be utilized subsequently in the composition of the paper, so that the loss in weight is immaterial and the result is a very large yield.

50 Moreover, the pieces are more or less saturated with the solution, which solution

is further utilized in the performance of the second treatment of my method.

The solution is then drawn off or removed. The same solution may be used repeatedly 55 as a softening agent for a large number of times, if desired, and in such case it becomes quite rich in potash which is extracted from the cellulosic substance sufficiently to admit of the potash being claimed by evaporation or other means for commercial purposes.

The second treatment; The mass having been thus treated is then cooked with a bisulphite pulp forming liquor, or a sodium 65 chloride solution depending upon which kind of paper the pulp is to be used for.

For instance, when during the first treatment a sodium chloride solution is employed, then, during the second treatment a bisulphite liquor may be employed and pulp for a fine grade of paper will be produced 70 which will be suitably bleached.

The strength of the bisulphite solution 75 will be such, together with the time and temperature of cooking that the fiber will not be destroyed outside of the fiber walls as usually is the case in the ordinary processes.

The first treatment only softens the 80 ligneous matter and the fiber and therefore a weak solution can be used on the second treatment thus retaining all the fiber in the material treated.

This second treatment may continue for a 85 period of time, say from 6 to 12 hours, at a temperature of from 110 degrees C. to 130 degrees C., but the longer the period of time and the lower the temperature, within reasonable limits, the better the pulp and larger 90 the yield.

There is a physical reaction between the softening agent, as sodium chloride, with which the mass is saturated during the first treatment, and the pulp forming agent employed as the bisulphite liquor employed during the second treatment, to which I attribute, at least in part, some of the advantages gained by this process.

On account of the first treatment, as afore- 100 said, a weaker pulp forming agent may be employed in the second cooking operation,

and also a lower temperature and a shorter period of time than under any of the methods known to me.

By this process a good news print paper may be produced with straw alone.

I claim:

1. The method of treating straw, corn-stalks and other cellulosic substances for the preparation of pulp for paper which consists in two successive treatments, first, treating the material with sodium chloride to soften but not destroy the ligneous matter, and second, cooking the treated mass with a bisulphite pulp forming liquor of such strength that the fiber will not be destroyed.

2. The method of treating straw, corn-stalks and other cellulosic substances for the preparation of pulp for paper which consists in treating the material with sodium chloride to soften but not destroy the ligneous matter and subsequently cooking the

mass with a bisulphite pulp forming liquor of such strength that the fiber will not be destroyed.

3. The method of treating straw, corn-stalks and other cellulosic substances for the preparation of pulp for paper which consists in two successive treatments, first, treating the material with sodium chloride to soften but not destroy the ligneous matter, and to extract potash from the cellulosic substance, then drawing off the softening agent containing the potash and then cooking the mass.

In testimony whereof, I have signed my name to this specification, in the presence of two subscribing witnesses.

CARL BACHE-WIIG.

Witnesses:

CHARLES M. DUMMOND,  
WADLEIGH B. DUMMOND.